

Aug. 30, 1938.

W. H. HARDING

2,128,482

METHOD OF PREPARING A SIZE

Filed June 25, 1935



INVENTOR.

WILLIAM H. HARDING,

BY  
Ellis S. Middleton

ATTORNEY.

## UNITED STATES PATENT OFFICE

2,128,482

## METHOD OF PREPARING A SIZE

William Harry Harding, Rockville Centre, N. Y., assignor to American Cyanamid & Chemical Corporation, New York, N. Y., a corporation of Delaware

Application June 25, 1935, Serial No. 28,259

5 Claims. (Cl. 134—21)

This invention relates to the manufacture of a composition of matter useful as a sizing material and constitutes an improvement upon the invention disclosed in co-pending application of John F. Fredriksson, Serial No. 571,990, filed October 30, 1931 now Patent 2,050,996.

In that application, it was proposed to dissolve caustic alkali in water as a saturated or supersaturated solution, dissipate the heat of solution and then mix the same with powdered rosin to produce a partially reacted mass as a direct dry product.

As an alternative procedure to the above, that application discloses the mixing of dry caustic alkali, water and rosin to accomplish the same effect.

Experience has demonstrated that if the caustic alkali, such as caustic soda is dissolved in water to make a saturated or supersaturated solution, such solution will salt out a part of the caustic at temperatures lower than 95° F. When rosin is ground prior to treatment with the caustic solution, it has been found desirable to refrigerate the same during the grinding period as this facilitates the grinding action. This refrigeration temperature is usually in the neighborhood of 60° F. and the rosin is delivered from the grinding equipment to the mixing equipment at substantially this refrigerated temperature. Under these circumstances, when the caustic solution meets the cold rosin, there is an appreciable precipitation of solid caustic from the solution. This precipitated material is of comparatively large size and, hence, causes an uneven distribution of the alkali through the rosin with which it is being mixed. This produces difficulties all along the line. When a caustic solution at 95° is sprayed upon the ground or crushed rosin, the added heat of the solution must be dissipated, together with the exothermic heat of reaction with the rosin and this, therefore, presents another objectionable feature of the above procedure. It is one of the principal objects of the invention to overcome the above objections.

Such salting out action can be prevented by maintaining the solution at a temperature elevated enough to maintain the caustic in solution even when it has been cooled by admixture with the relatively cold rosin but this is undesirable because it means that more heat must be dissipated to prevent detrimental heat effects. It is well known, of course, that if during the preparation of a resinate, high temperatures have been used, the floc resulting from the subsequent addition of alum to the resinate emulsion is darkened. This

darkened floc makes a size containing it useful only with certain types of paper or board and is not, therefore, universally useful. It is difficult to state the limits of this detrimental temperature, but it has been shown that a slightly elevated temperature maintained for a long time is equally as bad as a high temperature reached for only a comparatively short period. 5

It has been discovered that if a solution of caustic is made of a concentration such that its solids will not salt out at, say, 80° F. that more beneficial results are obtainable than has been possible heretofore. A solution of less than saturation at that temperature is more easily sprayed upon the ground rosin, making the necessity for a large nozzle orifice unnecessary, it is possible to use lower temperatures without getting into the floc darkening range, and less accumulated heat must be dissipated. Of course, if a solution of a concentration less than saturated is used, it means that for a given quantity of water, less alkali than is required to saponify an equivalent portion of rosin must be used. Where a completely saponified rosin product is eventually desirable, it is proposed to add an additional quantity of alkali in solid form and preferably ground to 80 mesh. 10 15 20 25

With the above objects in view, therefore, the invention, in one of its aspects, contemplates the use of a caustic alkali solution as a saponifying agent in concentrations which will not salt out at the normal room or operating temperatures commonly existent, to wit: in the neighborhood of 80° F. This concentration is short of saturation and the caustic alkali contained in such solution may be likewise short of an amount required to completely saponify the amount of rosin used. The additional quantity of alkali necessary for saponification, where desired, may be added to the rosin in the solid state, preferably pulverized to, say, 80 mesh. Of course, refrigeration may be resorted to to facilitate the crushing or grinding of both the rosin and the dry caustic alkali to be added thereto, although this is not necessary. 30 35 40

The invention further consists in the novel details more fully hereinafter described.

The drawing is a flow sheet illustrating a method employed.

In practice and to produce an ultimately completely saponified material, 14 pounds of caustic soda are required to completely saponify 100 pounds of rosin. In order to use only that quantity of water in the reaction to produce a solid product without going through the liquid stage, this caustic is ordinarily dissolved in 12 pounds 50 55

of water. As has been above stated, however, this quantity of alkali in the stated quantity of water gives a solution so saturated that it becomes supersaturated and salts out below 95° F.

5 In view of the above, it is preferred to dissolve less than 14 pounds of caustic alkali, say 12 pounds, in the equivalent of 12 pounds of water. This gives a solution so far from saturation as 10 will avoid this objectionable salting out at 80° F., yet making it possible to use this desirable 15 comparatively low temperature. The remaining two pounds of alkali, where a completely saponified product is desired, may then be added dry and preferably in a pulverized state of the fineness of 80 mesh to the powdered rosin. The alkali solution is either added to a mixture of powdered rosin and powdered dry alkali or the dry alkali may be added subsequently.

These proportions of solution alkali and dry 20 alkali may be varied, of course, dependent upon the temperature at which the mixing is to take place, that is, the lower the temperature used, the less concentrated should be the alkali solution and, where an ultimately completely saponified product is desired, the greater the quantity of the alkali added in the dry or solid state. Ordinarily, from 50% to 90% of the alkali should be added in solution form.

When the above operations are followed, the 30 alkali solution, the solid dry alkali and the rosin are thoroughly mixed, care being taken to avoid an undue rise in temperature. This may be accomplished by adding the solution, from which its heat of solution has been dissipated, slowly 35 as by spraying so as to permit the heat of reaction to be dissipated or a positive cooling effect may be obtained in the mixing apparatus by providing cooling elements. Ordinarily, the latter is not required.

40 As a result of the above operations, a direct dry product is obtained which microscopically has been found to consist of particles of solid caustic alkali and particles of solid rosin, coated either individually or collectively with dry sodium resinate. This coating prevents the absorption of 45 moisture by the dry alkali and consequent further reaction.

This dry product may be shipped in light 50 waterproof bags to the consumer and have been found to be remarkably stable and free flowing even under adverse conditions of humidity and pressure. The customer desiring to make a rosin size emulsion has only to add a quantity of this 55 material to a desired quantity of water and upon agitation the coating of resinate dissolves, thus liberating the dry rosin and caustic, which further react to produce a completely saponified

emulsion which is useful as a size for paper or the like.

In this application, where the word "caustic alkali" is used, it is to be understood as covering caustic soda, caustic potash, ammonium hydroxide, or in fact any material which will saponify rosin in appreciable quantities without the aid of heat. This qualification necessarily eliminates soda ash as a saponifying agent for a considerable amount of heat is required if this form of alkali is used and as has been above stated, at some length, heat is detrimental not only from the standpoint of cost because it requires additional equipment and a longer time element is involved, but also from the standpoint of a darkened floc.

I claim:

1. A method of preparing a dry composition of matter which includes mixing solid rosin, solid alkali and a solution of alkali the quantity of solid alkali used being greater than that which will dissolve in the solution of alkali at the mixing temperature, there being insufficient water to give a liquid product in which the total alkali used is sufficient to saponify the rosin, the dry alkali constituting from 10 to 50% of the total.

2. A method of preparing a dry composition of matter which includes mixing solid rosin, solid alkali and a solution of alkali the quantity of solid alkali used being greater than that which will dissolve in the solution of alkali at the mixing temperature, there being insufficient water to give a liquid product in which the total alkali used is sufficient to saponify the rosin, and of which from 90 to 50% is added in solution.

3. A method of preparing a dry composition of matter which includes mixing solid rosin, solid alkali and a solution of alkali the quantity of solid alkali used being greater than that which will dissolve in the solution of alkali at the mixing temperature, there being insufficient water to give a liquid product in which the dry and dissolved alkali is the same.

4. A method of preparing a dry composition of matter which consists in separately grinding 45 rosin and caustic soda to substantially 80 mesh, dissolving 12 pounds of caustic soda in 12 pounds of water, maintaining said solution at substantially 80° F., mixing 100 pounds of the ground rosin with two pounds of the ground caustic and spraying the caustic solution onto the mixture while agitating and while preventing any substantial rise in temperature.

5. The method of claim 4 in which the rosin is cooled to 60° F. during the grinding operation.

WILLIAM H. HARDING.